

## UNITED STATES PATENT OFFICE

2,229,030

## DRIVING JOURNAL COMPOUND

Elmer W. Adams, Hammond, Ind., and Lawrence C. Brunstrum, Chicago, Ill., assignors to Standard Oil Company, Chicago Ill., a corporation of Indiana

No Drawing. Application September 29, 1938,  
Serial No. 232,394

## 4 Claims. (Cl. 252—41)

This invention relates to lubricants of the driving journal compound type and particularly to such lubricants in which all or a large part of the soap content consists of soda soaps of certain low molecular weight fatty acids.

Lubricants of the driving journal compound type consist wholly or largely of soda soap and lubricating oil, the soda soap comprising from about 35% to about 55% and preferably from about 40% to about 50% of the product. The soap content of such products should be made from fatty acids rather than fats, i. e. should be substantially glycerine free and should also be substantially anhydrous although a trace of water is usually present.

In the past lubricants of the driving journal compound type have been made using soda soaps of fatty acid materials consisting almost wholly of fatty acids having at least 16 carbon atoms per molecule, for instance palmitic acid ( $C_{15}H_{31}COOH$ ), stearic acid ( $C_{17}H_{35}COOH$ ) or behenic acid ( $C_{19}H_{39}COOH$ ). We have found that greatly superior results can be obtained by the use of large amounts of soaps of fatty acids containing from 10 to 14 carbon atoms per molecule. We have found that lauric acid ( $C_{11}H_{23}COOH$ ) is particularly desirable, but myristic acid ( $C_{13}H_{27}COOH$ ) is also unusually good and capric acid ( $C_{9}H_{19}COOH$ ) can likewise be used to advantage. The 11 and 13 carbon atom saturated fatty acids ( $C_{10}H_{21}COOH$  and  $C_{12}H_{25}COOH$ ), while not found in nature in significant amounts, would no doubt share the advantages of the above materials.

It is an object of our invention to provide new and improved lubricants of the driving journal compound type and methods of manufacture therefor. Another object of our invention is to provide lubricants of the driving journal compound type having good body and high plasticity at room temperature coupled with very high softening times at elevated temperatures. A further object of our invention is to provide lubricants of the driving journal compound type having improved pressing characteristics. Another object of our invention is to provide a method of making lubricants of the driving journal compound type under steam kettle conditions which have properties even more advantageous than those of products which could be made heretofore only under the more drastic conditions of the fire kettle technique. Other and more detailed objects, advantages and uses of our invention will become apparent as the description thereof proceeds.

It is highly desirable that a lubricant of the driving journal compound type be plastic at ordinary temperatures so that it can be pressed into sticks or blocks and so that the formed lubricant will not break under conditions of use. At the same time it is very desirable that such lubricants retain their body at elevated temperatures so that they will continue to resist flow under low pressures. Otherwise these lubricants do not retain their form during use and are consumed too rapidly.

We find that these properties can be combined to a most unusual degree by the use of low molecular weight saturated fatty acids having from 10 to 14 carbon atoms per molecule. Such fatty acids can be made in a fairly high degree of purity by the fractional distillation of fatty acids obtained by the hydrolysis, and if necessary hydrogenation, of naturally-occurring fats.

Softening time is an index of quality from the service standpoint and is measured by a test in which a cylinder of driving journal compound  $\frac{1}{2}$  inch in diameter and about  $\frac{5}{8}$  inch long is heated on an oil or mercury bath to the desired test temperature while subjected to the weight of an 85 gram cylinder which provides a pressure on the driving journal compound comparable to the pressure to which the compound is subjected in actual operation when it is forced by a spring against a hot bearing. Softening time is defined as the time required to flatten the test cylinder one quarter of an inch under these conditions.

The following results show the softening times of lubricants of the driving journal compound type made in a steam kettle under like conditions using soda soaps of various fatty acids of about 90% purity:

| Soap used                                | Temperature |         | 40 |
|------------------------------------------|-------------|---------|----|
|                                          | 260° F.     | 300° F. |    |
|                                          | Seconds     | Seconds |    |
| Sodium stearate ( $C_{17}H_{35}COONa$ )  | 700         | 300     |    |
| Sodium palmitate ( $C_{15}H_{31}COONa$ ) | 600         | 300     |    |
| Sodium myristate ( $C_{13}H_{27}COONa$ ) | 12,000      | 1,000+  | 45 |
| Sodium laurate ( $C_{9}H_{19}COONa$ )    | Infinite    | 1,800+  |    |

In each case the driving journal compound tested had the composition:

|                                   | Per cent | 50 |
|-----------------------------------|----------|----|
| Soda soap                         |          | 45 |
| Steam refined oil (530° F. flash) |          | 45 |
| Heavy black oil                   |          | 10 |

The tests at 300° F. were not completed but at 55

1,000 and 1,800 seconds respectively the myristate and laurate samples were by no means completely flattened while the conventional products succumbed in 300 seconds. Still more startling are the results at 260° F. The myristate test sample was reduced in height only about  $\frac{1}{6}$  of the specified  $\frac{1}{4}$  inch in 2,000 seconds and the result is therefore given as 12,000 seconds. The laurate sample showed no tendency to soften at 260° F.

10 At the same time the myristate and laurate products were more plastic and more easily pressable at room temperatures than the stearate and palmitate products.

15 While best results are obtained by using soap containing at least about 85% of 10 to 14 carbon atom compounds excellent results can be obtained by using these low molecular weight materials in conjunction with greater quantities of soaps made from fatty acids of higher molecular weight. Thus the soap content of the driving journal compound can be from about 25% to 100% or better from about 50% to 100% soaps of 10 to 14 carbon atoms, the remainder being of higher molecular weight, for instance 16, 18 20 or more carbon atoms.

25 Lubricants in accordance with our invention can be made in accordance with any of the procedures known in the art by merely substituting the fatty acids above described for those heretofore used. However, these low molecular weight fatty acids can be used particularly advantageously in a steam kettle type of operation as contrasted with fire kettle technique and while fatty acids heretofore used to give low softening 30 time products when steam kettles are used this is not true when low molecular weight fatty acids are used.

35 In the steam kettle technique the soap is preferably formed in all of the oil at a temperature of from about 260° F. to about 300° F., but it can be formed in a portion of the oil under these con-

ditions and the remainder of the oil then graded in. In no case should the grease be heated above 330° F.

While we have described our invention in connection with certain preferred embodiments thereof, it is to be understood that these are by way of illustration and not by way of limitation and we do not mean to be bound thereby but only to the scope of the appended claims.

10 We claim:

1. In a substantially anhydrous lubricant containing from about 35% to about 55% soda soap, at least the bulk of the remainder being lubricating oil, the improvement which consists in using soda soap of which at least about 85% is made from saturated fatty acids having 12 carbon atoms per molecule.

2. In a substantially anhydrous lubricant containing from about 40% to about 50% soda soap, at least the bulk of the remainder being lubricating oil, the improvement which consists in using soda soap substantially free of unsaturated compounds of which at least about 85% is sodium laurate.

20 3. A substantially anhydrous lubricant of the driving journal compound type made up at least largely of soda soap and lubricating oil, said soda soap being substantially free of unsaturated compounds and containing at least about 25% of material having predominately 12 carbon atoms 30 per molecule, together with a substantial amount of soap having from 16 to 18 carbon atoms per molecule.

4. In a substantially anhydrous lubricant containing at least 25% soda soap, at least the bulk 35 of the remainder being lubricating oil, the improvement which consists in using soda soap of which at least about 85% is sodium laurate.

ELMER W. ADAMS.

40 LAWRENCE C. BRUNSTRUM.

CERTIFICATE OF CORRECTION.

Patent No. 2,229,030.

January 21, 1941.

ELMER W. ADAMS, ET AL.

It is hereby certified that error appears in the printed specification of the above numbered patent requiring correction as follows: Page 2, first column, line 34, strike out the word "to"; and second column, line 22, claim 2, strike out "substantially free of unsaturated compounds"; and that the said Letters Patent should be read with this correction therein that the same may conform to the record of the case in the Patent Office.

Signed and sealed this 25th day of February, A. D. 1941.

Henry Van Arsdale,  
Acting Commissioner of Patents.

(Seal)